

## UNITED STATES PATENT OFFICE

2,122,100

## PROCESS FOR COLORING AND WATER-PROOFING TEXTILE MATERIAL

Rudolf Kern, Oschatz, Germany, assignor to the firm Chemische Fabrik R. Baumheier Kommanditgesellschaft Oschatz-Zschöllau

No Drawing. Application December 13, 1933, Serial No. 702,259. In Germany December 15, 1932

2 Claims. (Cl. 91—68)

This invention relates to a process for simultaneously coloring and water-proofing textile materials in one bath. It has been found that the application of the dispersed water-proofing substances can be effected simultaneously with the coloring matter. The surprising discovery has been made that coloring matter or dyestuff and dispersed water-repelling particles do not impair each other's action in any operative phase, and that therefore, in spite of the presence of an emulsion, the coloring or dyeing takes place uniformly and not, as might be expected, irregularly, whereas for example uncleaned or unscooped cotton fibre containing a small quantity of wax, and readily repelling water, colors very irregularly, and in addition it is known that the parts of fibres coated with paraffin are not colored at all.

The surprising technical effect is that in spite of this a uniform coloring takes place. The process represents a very economical simplification of textile finishing since the operative time is considerably shortened, one operation being avoided. Thus the cost in manufacture is reduced considerably. After the dyeing it is not necessary to dry, before impregnating and then to dry again. The water-proofing emulsions are simply added to the coloring bath and the dyeing is effected in the usual way. The resulting wares are uniformly dyed and repel water to remarkable extent. The impregnation produced in this way will stand rinsing even in the case of moist articles, so that the auxiliary chemicals can be removed and in this manner subsequent damage to the fibre is avoided.

All emulsions used for water-proofing purposes may be employed, consisting of aqueous emulsions of water-proofing substances like paraffin, aluminium soaps, and so forth, or mixtures of such substances.

The following special emulsions also belong to emulsions of this type:

(1) *Aqueous emulsions of soaps of polyvalent metals*

The chief polyvalent metals are zinc, lead, magnesium, aluminium and copper. The acids which form soaps with these metals are fatty acids of the oleic and stearic acid type, or naturally occurring acid mixtures, such as, for example, acids of tallow, of palm oil, or of cocoanut oil, or acids of the resin acid type such as abietic acid.

Distinction is made between further subdivi-

sions of these emulsions, which relate to the production; they are subdivided into

- (a) those homogenized under pressure.
- (b) those emulsified in stirring machines, emulsifying machines or colloid mills.

14 parts of oil soap are stirred up with 15 parts of swollen bone glue and then diluted with water. This solution is stirred into 500 parts of a solution of formate of alumina having a specific gravity of 1.095. Thereupon 1-2% of hexane, butanol, acetic ester, acetone and the like are added. This emulsion is homogenized by forcing through ducts by means of suitable machines at a pressure of 60 atmospheres pressure.

(2) *Emulsions according to (1) both as regards composition and production, but characterized by the addition of water-proofing substances*

Water-proofing substances like paraffins, waxes, resins, fats, fatty oils or mineral oils may be used. Here also a distinction is to be drawn between emulsions which are

- (a) homogenized under pressure and
- (b) stated briefly, "emulsified".

By saponifying a mixture of 3.10 kg. of fatty acid with 4 kg. of mineral oil and 7.4 kg. of paraffin an emulsion is produced to which are added 1.29 kg. of high class glue dissolved in water. This substance is mixed with an aluminium formate solution which has been prepared by dissolving 1.55 kg. of 50% hydroxide of alumina in 1.75 kg. of 90% formic acid. The whole is then homogenized at 100 atmospheres pressure. At the concentration employed 50 kg. of a white paste are then obtained after cooling, a 2.5% solution of which is sufficient for impregnation purposes.

(3) *Emulsions of water-proofing substances which contain water-soluble salts of polyvalent metals, chiefly water-soluble aluminium salts, with a positive disperse phase*

All the above mentioned three groups of emulsions are acidic, and their disperse phase is positively charged. They all stabilize by means of colloids which swell in water, most advantageously however by means of glue and gelatin. All three groups of the said emulsions may contain wetting agents.

30 parts of good gelatin are swollen in 550 parts of water, the glue is melted by heating and, with the aid of stirring mechanism, a mixture of 110 parts of paraffin (flow point 54°), 20 parts of bleached Montan wax and 80 parts of paraffin oil are stirred in. Whilst further stirring in the hot, 80 parts of aluminium formate

dissolved in 400 parts of water are slowly added, and the mixture thereupon homogenized under pressure and then cooled down.

The emulsions according to (1) and (2) form  
5 the subject matter of U. S. Patent application  
No. 555,148 of April 8, 1931, (Fabric impregnated  
with dispersed substances, etc.).

10 (4) Emulsions having a negative dispersed part consisting of soap, glue, gelatin, starch, dextrin, aliphatic or aromatic sulphonate acids as emulsifying agent

The disperse phase consists of the waterproofing substances already mentioned above.

15 5 parts of glue are dissolved in 100 parts of water and to this solution are added 4 parts of the sodium salt of amylnaphthalene sulphonic acid. Into this emulsifying solution is stirred a mixture of 22 parts of paraffin, 4 parts of cetyl alcohol and 6 parts of olive oil. The whole is worked up in a colloid mill to a fine emulsion.

The process may be carried out by adding the waterproofing substance as such to the dye bath, for example in the case of substantive dyes or acid wool dyes. The water-proofing substance, however, may also be added to the individual treatment baths in the dyeing, for example to the copper bath, to the after-chroming bath, to the generating bath of naphthol dyes, to the vat or to the luminous mordant. In the latter case those emulsions are advantageously preferred which already contain aluminium salts. Such emulsions occur in commerce in gelatinous form and consist of aqueous aluminium formate solution as continuous phase, paraffin or paraffin-like substance as the disperse phase, and glue as stabilizing and gelatinizing agent. The following manufacturing receipt will illustrate the composition of the emulsion.

40 30 parts of good quality gelatin are swollen in  
550 parts of water; the glue is melted by heating  
and, by means of a stirring mechanism, a mix-  
ture of 110 parts of paraffin (flow point 54°), 20  
parts of bleached Montan wax and 80 parts of  
paraffin oil are stirred in. Whilst continuously  
45 stirring in the hot, 80 parts of aluminium for-  
mate dissolved in 400 parts of water are slowly  
added after which homogenization is effected  
under pressure and the whole then cooled down.

When using such emulsions in alkaline baths the aluminium formate for the purpose of avoiding precipitation of aluminium hydroxide, is converted into an alkali-stable complex form by addition of tartrates or other polyoxy-compounds. To the above emulsion, for example 3 kg. of sodium tartrate are added and the emulsion then neutralized or rendered alkaline with caustic soda. The statements made in respect of the above emulsions illustrate the composition only of one group of emulsions, which can contain the various substances compounded together in varying amounts. The use as well of the oils which are usual in dyeing operations, which consist of sulphonated fatty acids or aromatic substances, and which are used for wetting or equalizing purposes, does not impair the action of the impregnation.

*Example 1.—Substantive dyeing*

"Makko" fabric is treated with the following bath: Ten grams of a gelatinized emulsion are dispersed in 500 grams of a 1% tartaric acid solution. The emulsion used has the following composition:

80 parts of gelatin are dissolved in 1000 parts of water and a mixture of 40 parts of cake paraffin

and 40 parts of paraffin oil are emulsified therein. This emulsion is treated with formate of alumina of 7° Bé. The diluted emulsion solution is poured into a bath of the following composition:

|                                                                              | Parts | 5  |
|------------------------------------------------------------------------------|-------|----|
| Water                                                                        | 500   |    |
| Diamine black B H (Schultz Farbstofftabellen 7th edition, volume 1, No. 393) | 2     |    |
| Glauber's salt                                                               | 15    |    |
| Calcined soda                                                                | 15    | 10 |

The cotton fabric is introduced in this solution at 60° C. and, whilst thoroughly stirring, the whole brought to boiling, maintained at the boiling point for 20 minutes after which the fabric is rinsed, squeezed out and dried. The waterproof qualities are determined according to U. S. specification Serial No. 684,074, of July 8, 1933, (Method of and system for testing the imperviousness to water of impregnated textiles).

The following constants are used in the present 20 determination:

Reduction in height in the examination of  
 the cotton ..... cms. 30  
 Drop sequence ..... drops in 7 seconds. 10 25  
 Drop weight ..... mg. 125

The following drop values are obtained:

|                                                                                                                                                                                | Drops |
|--------------------------------------------------------------------------------------------------------------------------------------------------------------------------------|-------|
| Cotton dyed without water-proofing agent in<br>the dye bath-----                                                                                                               | 2 30  |
| Material impregnated in the usual way with<br>the waterproofing substance as previously<br>described diluted 1:100, i. e. as 10 g./litre,<br>impregnated 10 min. at 60° C----- | 14    |
| Dyed and impregnated as described above<br>in Example 1-----                                                                                                                   | 21 35 |

It follows from this that the water-proof quality when waterproofing in the dye bath is considerably higher than is produced by impregnating in the usual way. 40

In order to examine the fastness to rinsing and to prove that the impregnating substance adheres very firmly, the piece impregnated in the dye bath is to be boiled in pure water for 3 minutes and then dried. The imperviousness to water still amounted to 10 drops after this treatment. 45

*Example 2.—Chromina duestuif*

**Example 5. *Streaming agency***

| Cotton fabric is dyed in the following bath:                                     |  | Grams   |
|----------------------------------------------------------------------------------|--|---------|
| Water                                                                            |  | 1200 50 |
| Dianil chrome brown R (Schultz Farbstofftabellen 7th edition, volume 1, No. 682) |  | 2       |
| Calcined soda                                                                    |  | 10      |
| Glauber's salt                                                                   |  | 15      |
| Tartaric acid                                                                    |  | 4 55    |

The imperviousness to water amounts under the same conditions as in Example 1 to 3 drops, after-chromed at 60° C. for half an hour.—Drop value: 2 drops. 60

A parallel experiment has been then carried out in which 10 parts of the same gelatinous emulsion as in Example 1 were added to 1000 parts of bath, after which dyeing was effected at 60° C. for half an hour, and the material rinsed, 65 squeezed out and ironed.—Drop value: 19 drops.

After-chroming was then carried out in the following bath:

|                             | Parts |
|-----------------------------|-------|
| Water                       | 1150  |
| Copper sulphate             | 2.5   |
| Potassium dichromate        | 2.5   |
| Glacial acetic acid         | 5     |
| An emulsion as in Example 1 | 10    |

Drop value: 25 drops.

A piece of fabric treated in this way is boiled for 10 minutes. The imperviousness to water still amounted to 14 drops after this treatment.

*Example 3.—Basic dyestuffs*

Artificial silk is preliminarily mordanted with a 2% tannin solution, and after a considerable delay fixed during half an hour at 50° C. with a solution of aluminium salt-containing emulsion of 15 g. per litre. This emulsion has the following composition:

30 parts of good quality gelatin are swollen in 550 parts of water and the glue is caused to melt by application of heat; by means of a stirring mechanism a mixture of 110 parts of paraffin (flow point 54°), 20 parts of bleached Montan wax and 30 parts of paraffin oil are stirred in. Whilst further stirring in the hot a solution of 80 parts of aluminium formate dissolved in 400 parts of water are slowly added, and thereupon the whole is homogenized under pressure and then cooled down.

The material is then rinsed in the cold and squeezed out and after drying dyed for three quarters of an hour at 60° C. in a bath of 1000 parts of water, 2 parts of rhodamine B (Schultz, Farbstofftabellen, volume 1, 7th edition, No. 364) and 5 parts of glacial acetic acid, after which it is rinsed hot and cold in the usual manner, squeezed out, dried and ironed. The water repelling effect is very marked.

*Example 4*

Artificial silk is mordanted as in the above example, fixed, and then simultaneously dyed and impregnated with methylene blue (Schultz, Farbstofftabellen, 7th edition, volume 1, No. 1038). The bath has the following composition:

A solution of one gram of methylene blue R, 40 500 grams of water (50° C.) and 5 g. of glacial acetic acid are filtered into an emulsion of 10 g. of a substance according to Example 5 and 500 g. of water (50° C.). The material is then introduced at 50° C. and dyed for one hour at 60° C. It is then fixed in a 0.1% solution of tartar emetic (the treatment being effected for half an hour at ordinary temperature) and thereupon rinsed and dried. The water-repelling action of the material treated in this way is very good.

*Example 5.—Naphthol dyeing*

Cotton is bottomed for 30 minutes in a 0.2% solution of sodium naphtholate AS SW (beta-hydroxynaphthoic acid beta-naphthalide) and then rinsed and squeezed out. The fabric treated in this way is then introduced into a bath of the following composition:

|                                                                                                                                   | Parts |
|-----------------------------------------------------------------------------------------------------------------------------------|-------|
| Water                                                                                                                             | 1000  |
| Water-proofing emulsion made as described below                                                                                   | 10    |
| Fast red KB base (4-chlor-o-toluidine Schultz, Farbstofftabellen, 7th edition, volume 1, No. 82) dissolved in glacial acetic acid | 1     |
| After thorough stirring potassium nitrite dissolved in distilled water is added                                                   | 2     |

The emulsion referred to above is made as follows:

By saponification of a mixture of 3.10 kg. of fatty acid with 4 kg. of mineral oil and 7.4 kg. of paraffin an emulsion is obtained to which is added 1.29 kg. of high class glue dissolved in water. This substance is mixed with an alu-

minium formate solution which has been prepared by dissolving 1.55 kg. of 50% hydroxide of alumina in 1.75 kg. of 90% formic acid. Homogenization is then carried out at a pressure of 100 atmospheres. With the concentration employed 50 kg. of a white paste are obtained after cooling.

Generation of the dye is carried out for 30 minutes at 31° C.; the material is then twice rinsed, dried and ironed.

Drop value: 26 drops.

*Example 6.—Indigo vat*

White raw wool fabric is boiled out and introduced into a bath of the following composition:

|                                                                      | Parts   |
|----------------------------------------------------------------------|---------|
| Water                                                                | 4500    |
| Sodium hyposulphite                                                  | 2.25    |
| Indigo (Schultz, Farbstofftabellen, 7th edition, volume 1, No. 1301) | 1.13 20 |
| Water-proofing emulsion made as in Example 5                         | 45      |
| Tartaric acid                                                        | 15      |

The impregnating substance, together with the tartaric acid, is neutralized by means of ammonia. The fabric is dyed in the usual way and after hanging awhile is dried. The value for the imperviousness to water for a falling height of 20 cms. amounted to 12 drops. Operations 30 are carried out in a similar manner with hydrone blue B (Schultz, Farbstofftabellen, 7th edition, volume 1, No. 1113).

*Example 7*

Skeined wool is dyed in the known manner by means of eriochrome red (Schultz, Farbstofftabellen, 7th edition, volume 1, No. 745) and thereupon afterchromed with potassium chromate in acid emulsion, which is made as follows:

14 parts of sodium oleate are stirred up with 15 parts of swollen bone glue and the whole diluted with water. This solution is then stirred into 500 parts of a solution of formate of alumina having a specific gravity of 1.095.

This emulsion is homogenized at 60 atmospheres pressure with the aid of suitable machines by forcing through ducts. The foregoing emulsion is diluted fourfold and represents the above emulsion in the condition for use, in which afterchroming is carried out. The skeined wool is satisfactorily water-repelling and can be worked up into water-proof articles of apparel.

When working in a suitable manner the uniformity of the dyeing is in all cases perfectly satisfactory. Since most impregnating agents are stabilized with glue or gelatin such products cannot be used for all dyeing processes, for example not in the presence of dyestuffs which act as tanning agents in acid solution. "Walk" yellow (Schultz, Farbstofftabellen, 7th edition, volume 1, No. 230) has been found to be such a dyestuff. This dyestuff acts in acid solution as a tanning agent, precipitates the glue and breaks down the emulsion. In this case emulsions are used which are stabilized for example by means of starch, dextrin, or mucilage. However, in any after-chroming bath which may be used, as in the after-chroming bath of Example 7, glue-containing emulsion may be used. Outstanding waterproofing effects are already produced when fractions of a gram of impregnating agent per litre are used. The impregnation described can be used in the known manner in all dyeing appliances or apparatus.

*Example 8.—Indanthrene vat*

A cotton fabric is treated at 60° C. in a hypo-sulphite vat of the following composition:

|    |                                                                                                                          |
|----|--------------------------------------------------------------------------------------------------------------------------|
| 5  | 15 g. of a substance                                                                                                     |
| 5  | 500 g. of water                                                                                                          |
|    | 2 g. of dyestuff (Indanthrene golden orange G double paste; Schultz, Farbstofftabellen, 7th edition, volume 1, No. 1245) |
| 10 | 3 g. of hyposulphite ( $\text{Na}_2\text{S}_2\text{O}_4$ )                                                               |
| 10 | 10 g. of common salt                                                                                                     |
|    | 5 g. of an emulsion of the following composition                                                                         |
| 15 | 1.5 kg. of 50% aluminium hydroxide                                                                                       |
|    | 2.1 kg. of formic acid                                                                                                   |
|    | 375 kg. of water                                                                                                         |
|    | 2 kg. of tartaric acid                                                                                                   |
|    | 7 kg. of concentrated ammonia                                                                                            |
|    | 99 kg. of paraffin                                                                                                       |
| 20 | 30 kg. of an oil fatty acid                                                                                              |
|    | 10 kg. of potash lye (45° Bé.)                                                                                           |
|    | 20 kg. of glue                                                                                                           |

The fabric is dyed for one hour at about 60° C., rinsed, soaped in a 0.5% soap solution containing 1% of the above emulsion, and rinsed once warm and twice cold. Five ccs. of an alumina solution of 7° Bé. are added per litre of the last rinsing bath. For a falling height of 30 cm. the waterproof value amounts to 21 drops. 5

What I claim is:-

1. A method of simultaneously and uniformly dyeing and waterproofing textile materials, comprising treating said materials in usual alkaline dyestuff bath containing also a stable emulsion of substantially colorless water-repellent substances and aluminium formate and a substance selected from a group consisting of tartaric acid 15 and tartrates, added for the purpose of converting the aluminium salt into a complex compound.

2. The method of claim 1, as modified in that the "tartrate" recited therein is tartaric acid.

20

RUDOLF KERN.